

2,694,044

## STABILIZATION OF PHOSPHOSULFURIZED HYDROCARBONS

Fred B. Fischl, Springfield, and Elmer B. Cyphers, Cranford, N. J., assignors to Standard Oil Development Company, a corporation of Delaware

No Drawing. Application December 8, 1951,  
Serial No. 260,764

10 Claims. (Cl. 252—32.7)

The present invention relates to additives for use in oils and the like. It relates particularly to phosphorus- and sulfur-containing compositions designed to improve lubricating oils, greases, and the like.

The prior art recognizes the fact that lubricants containing phosphorus and sulfur, among other things, are capable of carrying higher unit loads without failure of the lubricating film than are lubricants which do not contain these elements. For example, certain hydrocarbon oils, such as "bright stock" lubricating oils and related mineral lubricating oil base stocks, may be treated at relatively high temperatures with various phosphorus sulfides, especially  $P_2S_3$ , although  $P_2S_3$ ,  $P_4S_3$  and  $P_4S_7$  and others or mixtures of these may also be used. Treatment is continued long enough to add substantial sulfur and phosphorus. The resulting reaction products have been stabilized by treatment with bases, basic reacting materials, reactive olefinic hydrocarbons and the like. These materials stabilize lubricants containing the phosphorus sulfide-treated additive, reducing their corrosiveness toward copper, reducing their tendency to evolve hydrogen sulfide ( $H_2S$ ) and improving their odor.

The various methods of stabilizing phospho-sulfurized materials, however, have as yet failed to provide a complete answer to the problem of  $H_2S$  evolution. For example, it is frequently desired to store for considerable periods of time either the phospho-sulfurized material or oil concentrates of it prior to blending it into a finished lubricant. Excessive  $H_2S$  evolution often occurs during storage even though the material has been stabilized with one of the afore-mentioned treating agents. Furthermore, lubricants containing certain of the treated additives will under some conditions evolve  $H_2S$ . This tendency leads to corrosion and odor difficulties, impairs the saleability of the product, and makes the lubricants unsuitable for use in some types of engines.

It has been found, in accordance with the present invention, that the tendency of phospho-sulfurized lubricants to evolve hydrogen sulfide under storage conditions may be appreciably reduced by the presence of minor, inhibiting amounts of certain organic esters. These esters improve the stability of the phospho-sulfurized materials per se and of their derivatives. The esters also effect improvements when the phospho-sulfurized material is used as an additive in lubricants in small concentrations.

The organic esters used are unsaturated alcohol esters of monocarboxylic, aliphatic acids. They may be prepared by conventional means by esterifying the acid with a monohydric, unsaturated alcohol. For the purposes of the following description and claims, the terms "unsaturated alcohol" or "unsaturated ester" will refer to those having alcohol hydrocarbon radicals with at least one double bond. The double bond may be of the olefinic or aromatic type. The alcohol molecule may contain up to three, four or even more double bonds and preferably contains no acetylenic-type triple bonds.

The organic acids used in preparing the esters are preferably fatty acids in the lower molecular weight range, usually having below about 10 and preferably below about 6 carbon atoms. Typical acids are formic, acetic, propionic, isobutyric, n-valeric, and the like.

The unsaturated alcohols employed in preparing the esters may be primary, secondary or tertiary alcohols having the formula  $ROH$  wherein the R radical is a hydrocarbon radical having at least 2 carbon atoms. Prefer-

ably, R will have no more than about 15, more preferably below 10, carbon atoms. R may be an alkenyl (olefinic), dialkenyl (di-olefinic), cycloalkenyl (cyclo-olefinic), alkaryl, or alkenylaryl or the like radical. Typical alcohols include vinyl alcohol; allyl alcohol; geraniol; citronellol; benzyl alcohol; cinnamyl alcohol; 1-propyl, 1-phenyl alcohol; 1-pentene-3-ol; 3-butene-2-ol; m-methylbenzyl alcohol, and the like.

Unexpectedly, it has been found that neither the organic acid nor the alcohol alone is effective for inhibiting  $H_2S$  evolution. Furthermore, the alcohol ester radical must be unsaturated or aromatic since the saturated alcohol ester of an unsaturated aliphatic acid is ineffective. For example, cinnamic acid, ethyl cinnamate, geraniol and benzyl alcohol are inactive in suppressing  $H_2S$  evolution from phosphosulfurized lubricants. Benzyl acetate, geranyl acetate and the like are, on the other hand, quite effective. An ester of an unsaturated aliphatic acid may be used providing the ester radical derived from the alcohol is also unsaturated.

While the position of the double bonds in the unsaturated ester is not particularly critical, greater effectiveness is afforded by using a compound having at least one double bond separated from the carbonyl oxygen by at least one  $CH_2$  group and such compounds are preferred. However, those having a double bond in a conjugated, alpha-beta position with respect to the carbonyl oxygen may be used effectively.

The phosphosulfurized hydrocarbon is prepared by treating a substantially olefin-free hydrocarbon, having a viscosity above about 50 Saybolt seconds Universal (S. S. U.) at 210° F. with a substantial proportion of a phosphorus sulfide at an elevated temperature. The proportions of the phosphorus sulfide may vary from as little as 5% to as much as 25%, the preferred range being around 10% to 20% of the phosphorus sulfide based on the weight of the oil. The treating temperature employed is in the range of 375° to 475° F., preferably in the range of 400 to 430° F. The hydrocarbon obviously must be of such type, including viscosity and boiling point, that it remains stable during the treatment. The time of treatment may vary somewhat, from as little as 1 hour to as much as 20 hours or more. The reaction is preferably continued for several hours, for example 10 hours or so and until the oil has a phosphorus content of 2 to 4% or more by weight and a sulfur content of 5% or more by weight. The phosphorus content may be as high as 5 or 6% and the sulfur content as high as 10 to 12%, but treatment should not be extended to the point that the material becomes insoluble in the oil base stock in which it is to be used. Ordinarily the upper limit is about 5 to 6% for the phosphorus content and about 9 to 11% for sulfur.

Preferred hydrocarbons for phosphosulfurization are lubricating oil base stocks such as bright stocks having for example an S. S. U. viscosity at 210° F. in the range from about 120 to 250 Saybolt seconds. They may be obtained, for example, by deasphalting, dewaxing, acid-treating, clay-treating, etc., of various petroleum residua. The higher molecular weight paraffins, aromatics, cyclic aliphatics, alkaryl compounds, and the like, may be used. Petrolatums, waxes, solvent extracts of petroleum fractions, etc., are also suitable. On the other hand, the unsaturated esters are generally ineffective in inhibiting  $H_2S$  evolution from phosphosulfurized olefinic materials such as those derived from terpenes.

The unsaturated ester of the present invention may be added to the phosphosulfurized hydrocarbon or to an oil concentrate before storage or shipment. However, the hydrocarbon treated in the manner described normally shows a titratable acidity and is highly objectionable because of its fairly high degree of instability. In order to reduce this instability, which is evidenced also in a high degree of corrosivity toward copper and objectionable odor, the reaction product of the hydrocarbon and phosphorus sulfide is preferably at least partially stabilized by further treatment before adding the unsaturated ester.

For example, the phosphosulfurized oil may have a portion or substantially all of its titratable acidity neutralized by treatment with a suitable basic reacting com-

product. Such compounds include the hydroxides, carbonates, or oxides of alkali or alkaline earth metals, such as potassium or sodium hydroxide, lime, barium hydroxide, and the like. Other basic reagents such as ammonia, alkyl or aryl substituted ammonia, such as amines or guanidine and derivatives thereof, or other neutralizing agents may be used. This reaction may be carried out by treatment with the basic reagent in solid or solution form using elevated temperatures up to about 400° F. The phosphosulfurized material may also be treated with an esterifying agent such as an alcohol, phenol, mercaptan or the like.

If desired, the phosphosulfurized product may be reacted with minor proportions, about 2 to 50 weight per cent based on the total material, of a suitably active olefinic hydrocarbon. By "suitably active" is meant that the olefinic material has the property of reacting with loosely bound sulfur in the phosphosulfurized oil in order to help stabilize the composition against subsequent H<sub>2</sub>S evolution. The preferred olefinic hydrocarbon materials to be reacted with the phosphosulfurized material include the terpenes, terpineol, and the like and such olefinic hydrocarbons as isobutylene, diisobutylene and the more reactive of the analogous aliphatic and cycloaliphatic materials. In particular, a product sold commercially as "Dipentene" consisting primarily of a mixture of true dipentene with its isomers and minor proportions of related products, may be used.

The ingredients may be mixed together and heated at a suitable temperature until a product of improved stability is obtained. The soaking temperature and the soaking time will vary depending upon the particular ingredients used and upon the degree of stability required. In general soaking temperatures from as low as 60° to as high as about 400° F. and soaking times of from 1 to 10 hours may be employed, depending upon the tendency to evolve H<sub>2</sub>S gas and upon the degree of stability desired. More broadly, the time required for soaking may be as little as one-quarter of an hour to as much as 20 hours.

The amount of unsaturated ester added may be varied within the general range of about 0.1 to 5.0 weight per cent, based on the treated or untreated phosphosulfurized hydrocarbon. A preferred range is about 0.5 to 2.0 weight per cent. The phosphosulfurized hydrocarbon is added to lubricants or greases in amounts ranging from about 0.1 to 20.0 weight per cent, based on the lubricant, the specific amount depending on the ultimate use of the lubricant. For example, amounts below about 5.0 weight per cent will generally suffice if detergency properties are needed. Proportions in the range of 5 to 20 weight per cent may be needed for gear lubricants and the like for extreme pressure service.

The phosphosulfurized additive may be stored and shipped as such or in the form of a concentrate in an oil base stock containing from about 20 up to 50 or more weight per cent of the active ingredient. The concentrate is then used for dilution with the finished lubricant or grease.

The unsaturated ester may be added to the finished viscous lubricating oil after the phosphosulfurized material has been blended therein, particularly if the latter material is added to lubricants shortly after phosphosulfurization. The present invention has particular application, however, to the inhibition of the concentrated, treated or untreated phosphosulfurized material.

The invention will be further illustrated by reference to the following examples:

#### Example

A deasphalted, dewaxed, acid- and clay-treated Panhandle bright stock having an S. S. U. viscosity of about 170 at 210° F. was treated in a nitrogen atmosphere with 17.5 weight per cent, based on the oil, of PaS for 10 hours at a temperature of 425° F. The product was then filtered and was found to have phosphorus and sulfur contents of about 3.5 and 6.5 weight per cent, respectively. The above phosphosulfurized oil was then treated with 9.5 weight per cent of commercial dipentene at a temperature of 380° F. with stirring for 1.0 hour. Commercial "dipentene" contains about 31% dipentene, 39% terpinolene, 6% alpha-pinene, 10% para-cymene, 7% alpha terpene, 5%  $\Delta_2,4(8)$ -p-menthadiene, and 2% residue. The material was then cooled to room temperature while blowing with nitrogen.

Product A was prepared by blending with the treated material 0.17 weight per cent of oil-soluble sodium petroleum sulfonate having a molecular weight of about 500 and 0.67 weight per cent of barium tert-octyl phenol sulfide.

Blends of Product A containing 1.0 weight per cent concentrations of various alcohols, acids, and esters were then prepared and tested for H<sub>2</sub>S evolution tendencies as follows: Four-ounce bottles were filled about three-fourths full with the product and stoppered with a tin foil-covered cork. The bottle was then stored at room temperature. Periodically, the stoppers were removed, and a filter paper that had been dipped in saturated lead acetate solution just prior to the test was placed over the bottle opening. After 30 seconds, the test papers were removed, dried, and given an "H<sub>2</sub>S Rating" by comparison with a set of standards in which "0" represents no stain and "10" represents a heavy, black, metallic stain. Product A was also tested for purposes of comparison. The data are as follows:

|                        | Storage Time, Days | H <sub>2</sub> S Rating |     |     |     |
|------------------------|--------------------|-------------------------|-----|-----|-----|
|                        |                    | 1                       | 3   | 6   | 20  |
| Compound in Product A: |                    |                         |     |     |     |
|                        | None               | 6                       | 9   | 10+ | 10+ |
| 30                     | Acetic Acid        | 10+                     | 10+ | 10+ | 10+ |
|                        | Vinyl Acetate      | 6                       | 7   | 7   | 7   |
|                        | Benzyl Alcohol     | 10                      | 10  | 10  | 10+ |
|                        | Benzyl Acetate     | 5                       | 4   | 6   | 7   |
|                        | Geraniol           | 8                       | 10+ | 10+ | 10+ |
|                        | Geranyl Acetate    | 4                       | 3   | 3   | 5   |
|                        | Cinnamic Acid      | 10                      | 10  | 10  | 10+ |
| 35                     | Ethyl Cinnamate    | 10                      | 10  | 10  | 10+ |

The phosphosulfurized bright stock, even after treatment with dipentene, was unstable in its undiluted state. Various organic acids and alcohols were ineffective for suppressing H<sub>2</sub>S evolution or even tended to increase H<sub>2</sub>S evolution. The addition of esters derived from unsaturated alcohols gave prolonged protection. It should be emphasized that the above ratings are on the phosphosulfurized material per se, and that the improvements obtained were sufficient to bring the rating of a finished lubricant containing relatively small amounts of the phosphosulfurized hydrocarbon to desirable low values.

It will be obvious to the skilled workman that other additives in addition to the additives mentioned heretofore may be used in the finished lubricant. Such additives include thickeners, viscosity index improvers, oxidation inhibitors, metal deactivators, pour point depressants and the like.

What is claimed is:

- An additive composition for lubricants comprising a major portion of a phosphosulfurized, substantially non-olefinic hydrocarbon and stabilizing amounts of an ester of an aliphatic acid having less than about 6 carbon atoms and a monohydric, unsaturated alcohol having at least 2 and less than 10 carbon atoms, said amounts being sufficient to stabilize the material against substantial evolution of sulfur containing gases.
- A composition in accordance with claim 1 wherein said acid is a fatty acid.
- An additive for lubricants comprising a stabilized phosphosulfurized mineral lubricating oil base stock containing at least 2 weight per cent phosphorus and 5 weight per cent sulfur and minor quantities of an ester of a monocarboxylic acid having less than about 6 carbon atoms and a monohydric alcohol having at least one double bond and from 2 to less than 10 carbon atoms in the molecule sufficient to stabilize the material against substantial evolution of sulfur-containing gases.
- A composition in accordance with claim 3 in which said phosphosulfurized oil has been stabilized by the addition of a basic reacting compound.
- A composition in accordance with claim 3 in which said phosphosulfurized oil has been stabilized by treatment with a reactive olefinic hydrocarbon.
- A composition in accordance with claim 5 in which said acid is acetic acid.
- A composition in accordance with claim 3 in which said alcohol is geraniol.
- A composition in accordance with claim 3 in which said alcohol is benzyl alcohol.

9. A composition in accordance with claim 3 in which said alcohol is vinyl alcohol.

10. An additive composition for lubricants comprising a major portion of a phosphosulfurized, substantially non-olefinic hydrocarbon and stabilizing amounts of vinyl acetate said amounts being sufficient to stabilize the material against substantial evolution of sulfur-containing gases.

## References Cited in the file of this patent

## UNITED STATES PATENTS

|   | Number    | Name         | Date          |
|---|-----------|--------------|---------------|
| 5 | 2,386,952 | Hughes       | Oct. 16, 1945 |
|   | 2,593,496 | Smith et al. | Apr. 22, 1952 |